

## UNITED STATES PATENT OFFICE

2,414,327

METHOD OF WATER- AND SUNPROOFING  
PAPER AND TEXTILES AND THE COMPOSI-  
TION TO BE USED IN THE METHOD

Alvis R. Patterson, Port Saint Joe, Fla.

No Drawing. Application September 3, 1941,  
Serial No. 409,381

16 Claims. (Cl. 106—287)

1

This invention relates to the treatment of textiles, paper and other fibrous materials.

One object of the invention is a novel and improved composition of materials or chemicals for treating textiles, paper and other fibrous materials for the purpose of imparting to them water-proof qualities.

A further object of the invention is a composition of the character indicated above which improves the qualities of said fibrous materials when treated according to the methods herein set forth.

A further object of the invention is a novel and improved method of treatment of fibrous materials in order to improve their waterproofing qualities.

A further object of the invention is a novel and improved method of treatment of fibrous materials in order to improve their sunproof qualities.

I have found that textiles, paper and other fibrous materials may be substantially improved in quality and their waterproofing qualities enhanced by treating them with a composition or mixture of chemicals containing ferrous sulphate ( $FeSO_4 \cdot 7H_2O$ ), phosphoric acid and a suitable alkali, such as pure soap or black liquor, and particularly when these constituents or ingredients are incorporated in the proportions or range of proportions indicated below.

The relative proportions of these ingredients may be varied within prescribed limits and I have found that a composition or mixture particularly suitable for textiles of from 3 to 30 grams of ferrous sulphate, .3 to 1 gram of phosphoric acid and .1 to 5 grams of alkali may be used to advantage.

I have found suitable a composition consisting of 30 grams of ferrous sulphate, 1 gram of phosphoric acid and 1 gram of ordinary pure soap (as for example Ivory soap), all included in solution in one quart of water.

The range of proportions given above for textile fabrics applies generally to paper.

To obtain the desired colors of the textile fabrics and papers, dyes may be applied to the solution, which solution will then color and waterproof the textile fabric or paper fabric at the same time. In so doing, it is not necessary to use fast dyes for the waterproofing makes a non-fast dye fast.

The textile fabric or paper fabric may be treated with the composition or mixture either by dipping the same in a bath of the composition, or the composition may be applied to the textile or paper fabrics in any suitable manner, as, for example, by pouring or spreading the composition on one side or both sides, as may be desired. The

2

fabrics do not need to be subjected to the composition for any considerable period since they rapidly absorb the composition. Textile fabrics after being so treated may be washed in hot water with the conventional washing powders and soaps or cleaned with cleaning fluids and when dried will again be water resistant.

I have found my novel and improved composition as particularly adapted to the waterproofing of non-sized paper such as 9 point (.009) board, etc. By the treatment of 9 point board and the like with a composition generally consisting of

10 Ferrous-sulphate \_\_\_\_\_ grams 5  
85% phosphoric acid \_\_\_\_\_ cc .07  
15 Soap flakes \_\_\_\_\_ grams .25

or  
Weak black liquor of about 8° Baumé, from the sulphate process of making pulp \_\_\_\_\_ grams 1

20 Dissolved in enough ordinary water to make 1000 cc. of solution.

I have very substantially increased its waterproof qualities.

25 While I have found phosphoric acid as the preferred acid generally to be incorporated in the composition, other acids may be employed with fairly good results, such as tannic, citric, lemon juice, tartaric, phormic, etc. I prefer ordinary pure commercial soap such as Ivory soap, or black liquor (such as used in the sulphate process for making paper), although other alkalies may be employed, such as sodium hydroxide, etc.

The following are other examples of suitable 30 formulae.

For paper, textiles, and wood, a composition of the following proportions is quite satisfactory:

35 Ferrous-sulphate ( $FeSO_4 \cdot 7H_2O$ ) grams 3 to 10  
85% Phosphoric acid \_\_\_\_\_ cc .04 to .1  
Soap flakes (Ivory preferred) \_\_\_\_\_ grams .5 to 6.0

Weak black liquor of about 12° Baumé from the sulphate process of making pulp \_\_\_\_\_ grams .8 to 5

40 Dissolved in enough water to make 1000 cc. of solution.

A still more specific and preferred composition for these purposes is as follows:

45 Ferrous-sulphate ( $FeSO_4 \cdot 7H_2O$ ) grams 5  
85% phosphoric acid \_\_\_\_\_ cc .07  
Soap flakes (Ivory preferred) \_\_\_\_\_ grams 1

or  
Weak black liquor of about 12° Baumé from the sulphate process of making pulp \_\_\_\_\_ grams 2

50 Dissolve the above in enough ordinary water to make 1000 cc. of solution.

This formula figures out roughly in percentages—

|                                                                               | Percent |
|-------------------------------------------------------------------------------|---------|
| Ferrous-sulphate ( $FeSO_4 \cdot 7H_2O$ )                                     | .5      |
| 85% phosphoric acid                                                           | .007    |
| Soap flakes (Ivory preferred)                                                 | .1      |
| or                                                                            |         |
| Weak black liquor of about 12° Baumé from the sulphate process of making pulp | 2       |
| Ordinary water if soap flakes are used                                        | 99.393  |
| or                                                                            |         |
| Ordinary water if black liquor is used                                        | 99.293  |

Experience has shown that the following specific composition is especially good for paper, although applicable to textiles and wood also:

|                                                                  |       |     |
|------------------------------------------------------------------|-------|-----|
| Ferrous-sulphate ( $FeSO_4 \cdot 7H_2O$ )                        | grams | 5   |
| 85% phosphoric or tartaric acid                                  | cc    | .07 |
| Tannic acid                                                      | grams | .2  |
| Weak black liquor                                                | do    | 2   |
| Dissolved in enough ordinary water to make 1000 cc. of solution. |       |     |

Lemon juice and the other acids mentioned above may be used instead of phosphoric or tartaric acid in about the same proportions as prescribed above. Tannic acid may be used in conjunction with phosphoric or tartaric to improve the gray color my process tends to give to paper, as indicated for example in the formula set forth above. If sodium hydroxide is used instead of soap or black liquor it should be used in a weaker or smaller proportion, namely about one-half gram or .05%.

I may use two or more acid constituents but ordinarily I prefer to use only one acid, namely phosphoric acid, particularly for textiles.

In the treatment of paper, I have found the following composition particularly suitable:

|                                                                                              | Grams    |
|----------------------------------------------------------------------------------------------|----------|
| Tannic acid                                                                                  | 1        |
| Ferrous-sulphate                                                                             | 20 to 30 |
| Black liquor (such as used in the sulphate process for making paper) of about 1.8 to 3 Baumé | 2        |
| Citric acid                                                                                  | 1        |
| Phosphoric acid                                                                              | 1        |
| All included in solution in one quart of water.                                              |          |

For best results the mixture is heated to 150° F. or lukewarm temperature at time of application. The composition can be highly concentrated or made into a powder for facilitating the handling or merchandising of the same, and when the composition is formed of a powder the user need only introduce it into the specified quantity of water to thoroughly dissolve and mix the same.

Textile fabrics or paper fabrics may be colored without affecting the water resistant qualities as pointed out above. Textiles may be dyed either along with the process of treatment or afterwards but preferably along with the composition for economy of time and cost, and this applies also to paper.

My invention is also useful in the treatment of wood of all types, plastics and other cellulosic products for the purpose of making the same resistant to water, various other liquids, and mildew.

I have found that for best results the hydrogen ion concentration or pH of the solution should be from 3 to 7.5 with the preferred range being from 4.5 to 5.5. The exact chemical action or physical action of my composition in im-

proving the quality of articles is somewhat uncertain. However, it would appear that any free sulphuric acid hydrates or hydroxides that may form from ferrous sulphate are not required in waterproofing, and in fact any iron hydroxide that may form in the solution is generally a hindrance rather than a help, and by having the hydrogen ion concentration not much above neutral or on the acid side the formation of iron hydroxide to any appreciable degree is avoided. My experience indicates that hydrates and iron hydroxides will not impart any appreciable waterproof qualities to the fibrous materials. The ferrous sulphate is believed to be the principal constituent in the waterproofing function while the phosphoric acid or other acid employed hinders or limits the precipitation (which tends to cause spotting and streaking) and acts also as a stabilizer for the solution. The alkali, as for example soap to black liquor, functions to control or limit the pH, the other ingredients having a tendency to become too acid with age, when free sulphuric acid and other equivalent acids are liberated.

The black liquor or soap tends, therefore, to keep the solution at the right prescribed pH and helps to prevent the formation of these objectionable acids.

In certain instances I have used, in addition to the constituents above, a wetting agent, such as pine oil or alcohol but care has to be exercised in the control of the composition, otherwise the pine oil or alcohol is detrimental to the composition or solution. The heating of the composition or solution to about 150° F. or lukewarm temperature aids in penetration, making a wetting agent unnecessary, and the embodiments of the invention set forth above function best both for paper and textile fabrics when heated to about 150° before using.

Instead of forming the mixture, composition or solution of the ingredients mentioned above, the phosphoric acid and the ferrous sulphate may be mixed together in solution and the fabric treated with this mixture as a first step, and then as a second step, before the fabric is dry, the same is rinsed thoroughly in a soap or black liquor solution, and as a third step rinsed in clear water before drying. This rinsing is not necessary to waterproofing but it does help to improve color and tends to improve its waterproofing qualities to a certain extent. The preferred formula for this treatment, especially for textiles, is as follows:

|                                                                                                                                             |       |     |
|---------------------------------------------------------------------------------------------------------------------------------------------|-------|-----|
| Ferrous-sulphate ( $FeSO_4 \cdot 7H_2O$ )                                                                                                   | grams | 5   |
| 85% phosphoric acid                                                                                                                         | cc    | .07 |
| Dissolved in enough water to make 100 cc. of solution and heat to 150° or lukewarm. Soak cloth in this solution from 20 minutes to an hour. |       |     |

Prepare a solution of 1 gram soap flakes in water to make 1000 cc. solution. After cloth has soaked in the first solution from 20 minutes to one hour rinse thoroughly in the soap solution then in clear water and dry.

The application of the composition or solution to paper may be applied after the paper comes from the conventional paper machine. It may be applied, however, to the paper before it comes from the paper machine. As for example, it may be applied at the calender stacks or between any of the drier sections, whichever is more convenient to the type of paper machine using it, or it may be applied right after the paper leaves the paper machine wire before it reaches the drier

sections. The conventional sizing ingredients such as rosin, alum, etc., which are incorporated in the paper during the manufacture, will be either entirely left out or reduced considerably in quantity, according to the exact type of paper desired. The use of my composition results in a considerable saving in the cost of materials and in the cost of the manufacture of the paper.

In the practice of my invention as applied to the treatment of ordinary unsized paper board having specifications .009-26#, .012-33#-35#, .016-42#, .016-47# and .030-90#. I have increased their waterproof qualities very substantially as indicated by the following tests. The board was immersed in water and after two and one-half hours' continuous immersion in the water, it was withdrawn from the water and freed of excess water, and then weighed. Tests of around a hundred samples showed a gain in weight by such immersion of only from around 50% to 60% on the average. These results were obtained with finished paper board treated in accordance with my invention on both sides. Waterproofing qualities may be imparted to the paper board to a substantial degree by treatment of only one side of the board, as contrasted with similar board which had not so been treated. Paper and textile fabrics may thus have their waterproofing qualities substantially increased by treatment according to my invention on only one side, and where the use of such fabric involves exposure to moisture only on one side it may be desirable to treat such fabric only on the side to be thus exposed. I have also found that paper treated in accordance with the invention stands up better when subjected to the sun than papers not so treated and there is less tendency of the paper thus treated according to my invention to disintegrate upon being wet after a sun bake than with paper not treated according to my invention.

The use of my composition or process does not preclude the use of known waterproofing and sizing practices such, for example, as rosin sizing in the pulp and tub sizing with wax, etc., before, after, or along with treatment by my process. The added waterproofing and sunproofing qualities imparted to paper and the like by treatment under this invention probably result from the formation and deposit of ferrous oxide within the sheets, the ferrous oxide being insoluble in water and alcohol and the principal ingredients for effecting this result are the ferrous sulphate and the alkali, although it is understood that I am not bound by any theory of functioning of the composition and process. In treating paper the latter may be treated as stated above at the calender stacks or between the drier sections of the paper machine and the temperatures which in certain parts of the machine may reach 300° may also play a part in the chemical action, although quite satisfactory results have been obtained at temperatures below 300° as, for example, room temperatures.

I am aware of the fact that ferrous sulphate and other iron sulphates have been used or proposed to be used in the textile industry as mordants, etc., but I am not aware that my composition above set forth, or process of treatment, has ever been used or proposed to be used for the purpose of waterproofing and sunproofing textiles and papers.

I claim:

1. A composition for the treatment of textiles, paper and fibrous materials, comprising 3 to 10

grams ferrous sulphate, .3 to 3 grams of an acid of the group consisting of phosphoric, tannic, citric, tartaric, formic, and .8 to 5 grams of weak black liquor of about 12° Baumé derived from the sulphate process of making pulp.

2. A composition for the treatment of textiles, paper and fibrous materials, comprising 3 to 30 grams ferrous sulphate, and .3 to 3 grams of an acid constituent of the group consisting of citric, phosphoric, tannic, tartaric and formic, and an alkali in quantity from .1 to 5 grams.

3. A composition for the treatment of textiles, paper and fibrous materials comprising around 30 grams of ferrous sulphate, around 1 gram of phosphoric acid, and around 1 gram of soap dissolved in water.

4. A method of water-proofing textiles, paper and fibrous materials which consists in subjecting it to a solution containing from 3 to 30 grams of ferrous sulphate, .3 to 3 grams of an acid and from one-half to 6 grams of an alkali, said solution having a pH of from 3 to 7.5.

5. The method of water and sun-proofing paper and textile fabrics which consists in subjecting at least one side thereof to a solution containing 3 to 10 grams of ferrous sulphate as the basic ingredient, a fraction of 1 cubic centimeter of an acid and from  $\frac{1}{2}$  to 6 grams of an alkali, said solution having a pH of from 3 to 7.5.

6. A composition of chemical ingredients for the treatment of textiles, paper and fibrous materials containing 3 to 30 grams of ferrous sulphate, .3 to 3 grams of an acid and .1 to 5 grams of black liquor.

7. The method of waterproofing textiles, paper, and fibrous materials which consists in subjecting the same to a solution containing ferrous sulphate as the basic ingredient, an acid of the group consisting of phosphoric, citric, tannic, tartaric and formic, and an alkali and in the proportions of 3 to 30 grams of ferrous sulphate, .3 to 3 grams of the acid and  $\frac{1}{2}$  to 6 grams of the alkali, while maintaining the solution at a pH of from 3 to 7.5.

8. In a composition of the character set forth in claim 2 wherein the alkali is black liquor.

9. In a composition of the character set forth in claim 2 wherein the alkali is soap.

10. In a composition of the character set forth in claim 2 wherein the alkali is sodium hydroxide.

11. A composition of chemical ingredients for the treatment of textiles, paper and fibrous materials containing 3 to 30 grams of ferrous sulphate, three tenths of a gram to 3 grams of an acid, and one tenth of a gram to 5 grams of an alkali.

12. In the method of claim 5 wherein the paper fabric is treated with the solution after its formation and while it is passing through the dryer sections and calender stacks of the paper machine.

13. The method of water and sun-proofing paper and textile fabrics which consists in subjecting them to a solution containing ferrous sulphate in quantity sufficient to impart water and sun-proofing qualities thereto, with the pH of the solution at from 3 to 7.5 pH.

14. The method of water and sun-proofing paper and textile fabrics which consists in subjecting them to a solution containing ferrous sulphate in quantity sufficient to impart water and sun-proofing qualities thereto, with the pH of the solution at from 3 to 7.5 and then rinsing said fabrics with a dilute soap solution.

15. The method of water and sun-proofing textiles, paper and fibrous materials which consists in subjecting them to a composition of chemical ingredients in solution containing 3 to 30 grams of ferrous sulphate,  $\frac{1}{16}$  of a gram to 3 grams of an acid, and  $\frac{1}{16}$  of a gram to 5 grams of an alkali.

16. The method of water and sun-proofing

textiles, paper and fibrous materials which consists in subjecting them to a composition of chemical ingredients in solution containing approximately 5 grams of ferrous sulphate, a fraction of 1 gram of an acid, and from  $\frac{1}{4}$  of a gram to 1 gram of an alkali dissolved in water to form 1000 grams of solution.

ALVIS R. PATTERSON.